# EUROPEAN PATENT APPLICATION

(11) **EP 4 667 607 A1**
(43) Date of publication of application: **24.12.2025**
(21) Application number: 24779731.9
(22) Date of filing: 19.03.2024
(51) Int. Cl.: C22C 38/00, C21D 3/04, C21D 9/46, C22C 38/60, C23C 2/02, C23C 2/06, C23C 2/28

(54) **STEEL SHEET AND METHOD FOR MANUFACTURING STEEL SHEET**

(30) Priority: 30.03.2023 JP 2023056165; 19.02.2024 JP 2024022770
(71) Applicant: KABUSHIKI KAISHA KOBE SEIKO SHO (KOBE STEEL, LTD.), Hyogo 651-8585 (JP)
(72) Inventor: Maekawa, Shuya, Hyogo 651-2271 (JP); Otomo, Ryosuke, Hyogo 651-2271 (JP); Irie, Hiroshi, Hyogo 651-2271 (JP); Hirai, Shoichi, Hyogo 651-2271 (JP); Kiguchi, Kentaro, Hyogo 651-2271 (JP)
(74) Representative: Müller-Boré & Partner Patentanwälte PartG mbB
(86) International application number: PCT/JP2024/010716
(87) International publication number: WO 2024/203606

(57) **Abstract**

A steel sheet, wherein, in a sheet thickness direction,
a position where a carbon concentration (mass%) is 50% of a bulk carbon concentration is in a region of 0.20% or more of the sheet thickness from a steel sheet surface, and
a position where a carbon concentration (mass%) is 90% of the bulk carbon concentration is in a region of 8.0% or less of the sheet thickness from the steel sheet surface.

## Description

### TECHNICAL FIELD

The present disclosure relates to a steel sheet and a method for manufacturing a steel sheet. In particular, the present disclosure relates to a high-tension steel sheet superior in bendability, and a method for manufacturing a steel sheet.

### BACKGROUND ART

Conventionally, improvement in the safety of an occupant in a vehicle has been required, and strength of a material of a vehicle body has been improved for such a purpose. Meanwhile, with the growing of the global warming problem or the like as background, the movement for improving the fuel efficiency of automobiles is accelerating. It is known that weight reduction of a vehicle body is effective for improving fuel efficiency.

To increase the strength of a steel sheet to realize weight reduction of a vehicle body, addition of Si or Mn is effective. However, during continuous annealing, Si and Mn are oxidized even in a reducing atmosphere in which oxidation of Fe does not occur, and oxides of Si and Mn are formed on the outermost surface of a steel sheet. The oxide of Si or Mn lowers wettability between molten zinc and a base steel sheet, for example, during a zinc-based plating treatment, and thus there has been a problem that bare spots frequently occur or plating adhesion is poor in a steel sheet with addition of Si or Mn.

To address the above problems, Patent Document 1 discloses a method for manufacturing a high-strength galvanized steel sheet superior in plating adhesion, workability, and fatigue resistance properties, in which a steel sheet is subjected to an oxidation treatment, and then reduction-annealing. In the oxidation treatment, in a first stage, the steel sheet is heated at a temperature of 400 to 750°C in an atmosphere having an O₂ concentration of 1000 ppm by volume or more and an H₂O concentration of 1000 ppm by volume or more, and, in a second stage, the steel sheet is heated at a temperature of 600 to 850°C in an atmosphere having an O₂ concentration of less than 1000 ppm by volume and an H₂O concentration of 1000 ppm by volume or more. In the reduction-annealing, in a heating zone, the steel sheet is heated at a heating rate of 0.1°C/sec or more to a temperature of 650 to 900°C in an atmosphere having an H₂ concentration of 5 to 30% by volume and an H₂O concentration of 10 to 1000 ppm by volume with a balance of N₂ and inevitable impurities, and thereafter, in a soaking zone, the steel sheet is soaked and held for 10 to 300 seconds with a temperature variation in the soaking zone of ±20°C or less in an atmosphere having an H₂ concentration of 5 to 30% by volume and an H₂O concentration of 500 to 5000 ppm by volume with a balance of N₂ and inevitable impurities.

### PRIOR ART DOCUMENT

### PATENT DOCUMENT

Patent Document 1: JP 2017-166057 A

### SUMMARY OF THE INVENTION

### PROBLEMS TO BE SOLVED BY THE INVENTION

In manufacturing an automobile component, a steel sheet may be bent into a component shape. However, a high-strength steel sheet having a strength of, for example, 980 MPa or more, or 1180 MPa or more has a problem that it is difficult to favorably perform bending thereon to obtain a desired component shape, that is, it is difficult to secure superior bendability. In Patent Document 1, improvement in the bendability of the plated steel sheet has not been studied. The present disclosure has been made in view of the above circumstances, and an object of the present disclosure is to provide a steel sheet having high strength, capable of contributing to weight reduction of a vehicle body, and exhibiting superior bendability, and a method by which the steel sheet can be easily manufactured.

### SOLUTIONS TO THE PROBLEMS

Aspect 1 of the present invention is
a steel sheet, wherein, in a sheet thickness direction,
a position where a carbon concentration (mass%) is 50% of a bulk carbon concentration is in a region of 0.20% or more of the sheet thickness from a steel sheet surface, and
a position where a carbon concentration (mass%) is 90% of the bulk carbon concentration is in a region of 8.0% or less of the sheet thickness from the steel sheet surface.

Aspect 2 of the present invention is
the steel sheet according to Aspect 1, wherein a maximum value of a carbon concentration (mass%) in a region up to 20 µm in the sheet thickness direction from a steel sheet surface is less than 70% of the bulk carbon concentration, and
a surface layer decarburization amount per millimeter of the sheet thickness on one surface of the steel sheet is 0.045 mol/m² or less.

Aspect 3 of the present invention is
the steel sheet according to Aspect 1 or 2, wherein
the steel sheet has a tensile strength of 980 MPa or more.

Aspect 4 of the present invention is
the steel sheet according to any one of Aspects 1 to 3, wherein a component composition satisfies:
C: 0.08 mass% or more and 0.30 mass% or less;
Si: more than 0.5 mass% and 3.0 mass% or less;
Mn: 1.5 mass% or more and 3.0 mass% or less;
Cr: 0 mass% or more and 1.0 mass% or less;
P: more than 0 mass% and 0.1 mass% or less;
S: more than 0 mass% and 0.05 mass% or less;
Al: more than 0 mass% and 1.0 mass% or less; and
N: more than 0 mass% and 0.01 mass% or less,
with the balance being Fe and inevitable impurities.

Aspect 5 of the present invention is
a method for manufacturing a steel sheet, the method comprising an annealing step of performing an oxidation treatment under conditions of an oxygen concentration of 0.1 to 2% and an attainment temperature of 650 to 750°C and then performing a reduction treatment,
wherein the reduction treatment is performed through a first reduction treatment having a dew point of -35 to -15°C, and subsequently through a second reduction treatment having a dew point being -25 to 0°C and being higher than the dew point of the first reduction treatment.

Aspect 6 of the present invention is
the method for manufacturing a steel sheet according to Aspect 5, wherein an attainment temperature in the first reduction treatment and the second reduction treatment is 800 to 920°C.

### EFFECTS OF THE INVENTION

According to the present disclosure, it is possible to provide a steel sheet having high strength, capable of contributing to weight reduction of a vehicle body, and exhibiting superior bendability, and a method for manufacturing the steel sheet.

### BRIEF DESCRIPTION OF THE DRAWINGS

[Fig. 1-1] Fig. 1-1 is a graph showing the relationship between the dew point at the center of the soaking zone during the second reduction treatment and R/t.
[Fig. 1-2] Fig. 1-2 is another graph showing the relationship between the dew point at the center of the soaking zone during the second reduction treatment and R/t.
[Fig. 2-1] Fig. 2-1 is a graph showing the relationship between the dew point at the center of the soaking zone during the second reduction treatment and the tensile strength TS.
[Fig. 2-2] Fig. 2-2 is another graph showing the relationship between the dew point at the center of the soaking zone during the second reduction treatment and the tensile strength TS.
[Fig. 3] Fig. 3 is a diagram showing one example of a carbon concentration profile obtained in Examples.
[Fig. 4-1] Fig. 4-1 is a graph showing the relationship between the position where the carbon concentration (mass%) in the sheet thickness direction is 50% of the bulk carbon concentration and R/t.
[Fig. 4-2] Fig. 4-2 is another graph showing the relationship between the position where the carbon concentration (mass%) in the sheet thickness direction is 50% of the bulk carbon concentration and R/t.
[Fig. 5-1] Fig. 5-1 is a graph showing the relationship between the position where the carbon concentration (mass%) in the sheet thickness direction is 90% of the bulk carbon concentration and the tensile strength TS.
[Fig. 5-2] Fig. 5-2 is another graph showing the relationship between the position where the carbon concentration (mass%) in the sheet thickness direction is 90% of the bulk carbon concentration and the tensile strength TS.
[Fig. 6-1] Fig. 6-1 is a graph showing the relationship between the ratio of the maximum value of the carbon concentration (mass%) in the region up to 20 µm from the steel sheet surface to the bulk carbon concentration and R/t.
[Fig. 6-2] Fig. 6-2 is another graph showing the relationship between the ratio of the maximum value of the carbon concentration (mass%) in the region up to 20 µm from the steel sheet surface to the bulk carbon concentration and R/t.
[Fig. 7-1] Fig. 7-1 is a graph showing the relationship between the surface layer decarburization amount per millimeter of the sheet thickness and the tensile strength TS.
[Fig. 7-2] Fig. 7-2 is another graph showing the relationship between the surface layer decarburization amount per millimeter of the sheet thickness and the tensile strength TS.

### DETAILED DESCRIPTION

The present inventors intensively studied to obtain a steel sheet exhibiting superior bendability during a bending work even with high strength. As a result, the present inventors have found that by providing a decarburized layer within a prescribed range in the steel sheet surface layer, superior bendability can be obtained with retention of high strength. In addition, the present inventors have found that controlling conditions for annealing a steel sheet (a substrate) can contribute to the formation of a decarburized layer within a prescribed range capable of achieving both high strength and superior bendability on a steel sheet surface layer. Hereinafter, the steel sheet of the present embodiment will be first described.

### [Steel Sheet]

### (Decarburized Layer of Steel Sheet Surface Layer)

In the steel sheet according to the present embodiment,
(I) in the sheet thickness direction,
   the position where the carbon concentration (mass%) is 50% of the bulk carbon concentration is in a region of 0.20% or more of the sheet thickness from the steel sheet surface, and
   the position where the carbon concentration (mass%) is 90% of the bulk carbon concentration is in a region of 8.0% or less of the sheet thickness from the steel sheet surface.

In the steel sheet according to the present embodiment, in the sheet thickness direction, the position where the carbon concentration (mass%) is 50% of the bulk carbon concentration is in a region of 0.20% or more of the sheet thickness from the steel sheet surface. The aforementioned positions relate to the thickness of the decarburized layer which contributes to bendability. When the position is in a region of 0.20% or more of the sheet thickness from the steel sheet surface, and a decarburized layer having a certain thickness or more that contributes to bendability is secured, superior bendability can be reliably exhibited in a bending work. The position where the carbon concentration (mass%) is 50% of the bulk carbon concentration may be in a region of 0.5% or more, or 1.0% or more of the sheet thickness from the steel sheet surface.

Furthermore, in the steel sheet according to the present embodiment, the position where the carbon concentration (mass%) is 90% of the bulk carbon concentration in the sheet thickness direction is in a region of 8.0% or less of the sheet thickness from the steel sheet surface. As the thickness of the decarburized layer increases, the bendability is improved, but the strength tends to decrease. As a result of examination by the present inventors, however, it has been found that a decrease in strength can be sufficiently inhibited when the position where the carbon concentration (mass%) is 90% of the bulk carbon concentration is in a region of 8.0% or less of the sheet thickness from the steel sheet surface. The position where the carbon concentration (mass%) is 90% of the bulk carbon concentration may be 6.0% or less of the sheet thickness from the steel sheet surface.

In the steel sheet according to the present embodiment,
(II) the maximum value of the carbon concentration (mass%) in a region up to 20 µm in the sheet thickness direction from the steel sheet surface is less than 70% of the bulk carbon concentration, and
the surface layer decarburization amount per millimeter of the sheet thickness on one surface of the steel sheet is 0.045 mol/m² or less, preferably 0.035 mol/m² or less.

As a result of confirming conventional steel sheets, the present inventors have first found that there is a region having a significantly high carbon concentration in the steel sheet surface layer, and this is a cause of deterioration in bendability. In addition, as will be described later, the present inventors studied conditions for manufacturing a steel sheet, and have found that when decarburization of the steel sheet surface layer is promoted to control the carbon concentration of the steel sheet surface layer, specifically, when the maximum value of the carbon concentration (mass%) in a region up to 20 µm from the steel sheet surface in the sheet thickness direction is controlled to less than 70% of the bulk carbon concentration, superior bendability can be easily obtained. The maximum value of the carbon concentration is preferably 65% or less of the bulk carbon concentration, and more preferably 60% or less of the bulk carbon concentration.

In addition, in the steel sheet according to the present embodiment, the surface layer decarburization amount per millimeter of the sheet thickness on one surface of the steel sheet is controlled to 0.045 mol/m² or less, preferably 0.035 mol/m² or less, whereby a tensile strength as high as 980 MPa or more, particularly 1180 MPa or more can be secured. The surface layer decarburization amount per millimeter of the sheet thickness is more preferably 0.030 mol/m² or less, and even more preferably 0.025 mol/m² or less.

From the viewpoint of achieving both high strength and superior bendability, the steel sheet according to the present embodiment is merely required to satisfy at least one of the above (I) and (II), and preferably satisfies the above (I), more preferably satisfies both the above (I) and (II).

The "steel sheet surface" refers to a surface of a steel sheet in the case of a steel sheet obtained by performing annealing on a cold rolled steel sheet, and refers to a position of the interface between a plating layer and a base steel sheet in the case of a plated steel sheet. For example, in the case of zinc-based plating, the position of the interface between the plating layer and the base steel sheet refers to a point where Zn constituting the plating layer is not detected (the analysis value of Zn becomes 0) when Zn is analyzed in the thickness direction of the plating layer from the surface of the plating layer by GD-OES performed in Examples described later, and this point is taken as the start point of the distance (depth) from the steel sheet surface.

The steel sheet according to the present embodiment exhibits superior bendability in a bending work even with high strength. As the strength, a tensile strength TS of 980 MPa or more, preferably 1180 MPa or more is exhibited, for example. In addition, the steel sheet according to the present embodiment exhibits superior bendability with a limit R/t of less than 2.5 when a bending test described in Examples described later is performed.

The sheet thickness of the steel sheet according to the present embodiment is not limited. The sheet thickness of the steel sheet according to the present embodiment (the sheet thickness of a base steel sheet in the case of a plated steel sheet) may be, for example, 0.4 mm or more and 4 mm or less.

### (Component Composition of Steel Sheet)

In achieving high strength, the steel sheet according to the present embodiment can have, for example, a Si content of more than 0.5 mass% in the component composition. The Si content is more preferably 1.0 mass% or more, even more preferably 1.1 mass% or more, and still even more preferably 1.2 mass% or more. The upper limit of the Si content may be, for example, 3.0 mass%.

As one preferred embodiment, the component composition of the steel sheet satisfies:
C: 0.08 mass% or more and 0.30 mass% or less;
Si: more than 0.5 mass% and 3.0 mass% or less;
Mn: 1.5 mass% or more and 3.0 mass% or less;
Cr: 0 mass% or more and 1.0 mass% or less;
P: more than 0 mass% and 0.1 mass% or less;
S: more than 0 mass% and 0.05 mass% or less;
Al: more than 0 mass% and 1.0 mass% or less; and
N: more than 0 mass% and 0.01 mass% or less,
with the balance being Fe and inevitable impurities. In the following, the respective elements are described.

### [C: preferably 0.08 mass% or more and 0.30 mass% or less]

C is an element effective for improving the strength of the steel sheet, and is a particularly effective reinforcing element for finally ensuring the tensile strength of the steel sheet of 980 MPa or more, or 1180 MPa or more, by being contained in the steel together with Si, and as necessary also with Mn. Furthermore, C is also an element necessary for securing retained austenite and improving the workability. To allow such an action to be effectively exerted, the C content is preferably 0.08 mass% or more, more preferably 0.11 mass% or more, and even more preferably 0.13 mass% or more. From the viewpoint of ensuring the strength of the steel sheet, it is preferable that the C content is larger, but when the C content is excessively large, corrosion resistance, spot weldability, and workability may be deteriorated. Therefore, the C content is preferably 0.30 mass% or less, more preferably 0.25 mass% or less, and even more preferably 0.23 mass% or less.

### [Mn: preferably 1.5 mass% or more and 3.0 mass% or less]

Mn is also an inexpensive steel reinforcing element, similarly to Si, and is effective for improving the strength of the steel sheet. Mn is a particularly effective reinforcing element for finally ensuring the tensile strength of the steel sheet of 980 MPa or more, or 1180 MPa or more, by being contained in the steel together with Si, and as necessary also with C. Furthermore, Mn is also an element that stabilizes austenite and contributes to improvement of the workability of the steel sheet due to the generation of retained austenite. To allow such an action to be effectively exerted, the Mn content is preferably 1.5 mass% or more, more preferably 1.8 mass% or more, and even more preferably 2.0 mass% or more. However, when the Mn content is excessively large, the ductility of the steel sheet decreases, which adversely affects the workability of the steel sheet, and there is a possibility that the weldability of the steel sheet decreases. From these points of view, the Mn content is preferably 3.0 mass% or less, more preferably 2.8 mass% or less, and even more preferably 2.7 mass% or less.

### [Si: more than 0.5 mass% and 3.0 mass% or less]

Si is an inexpensive steel reinforcing element, and hardly affects the workability of the steel sheet. In addition, Si is an element capable of suppressing the decomposition of retained austenite, which is useful for improving the workability of the steel sheet, into carbides. To allow such an action to be effectively exerted, the Si content is more than 0.5 mass%, preferably 1.0 mass% or more, more preferably 1.1 mass% or more, and even more preferably 1.2 mass% or more. The upper limit of the Si content is not particularly limited, but when the Si content is excessively large, a solid-solution strengthening action by Si is remarkable, leading to the risk that the rolling load increases. In addition, there is a possibility that a Si scale is generated during hot rolling to cause surface defects of the steel sheet. Therefore, for example, from the viewpoint of manufacturing stability, the Si content is preferably 3.0 mass% or less, more preferably 2.7 mass% or less, and even more preferably 2.5 mass% or less.

### [Cr: preferably 0 mass% or more and 1.0 mass% or less]

Cr is an element effective for improving the strength of the steel sheet. Furthermore, Cr is an element that improves the corrosion resistance of the steel sheet, and has an action of suppressing the generation of hydrogen due to the corrosion of the steel sheet. Specifically, Cr has an action of promoting the production of iron oxide (α-FeOOH). Iron oxide is said to be thermodynamically stable and protective among rusts produced in the atmosphere. By promoting the production of such a rust, it is possible to suppress the intrusion of generated hydrogen into the steel sheet, and it is possible to sufficiently suppress assisted cracking due to hydrogen even when the steel sheet is used under a severe corrosive environment, for example, in the presence of a chloride. In addition, because Cr is an element effective for the delayed fracture resistance of the steel sheet similarly to B and Ti, Cr can be contained in an amount at which the workability, such as strength or elongation, of the steel sheet is not affected. The Cr content may be 0 mass%, but to allow these actions to be effectively exerted, the Cr content is preferably more than 0 mass%, more preferably 0.003 mass% or more, and even more preferably 0.01 mass% or more. On the other hand, when the Cr content is excessive, there is a possibility that the workability, such as elongation, of the steel sheet is deteriorated. Therefore, the Cr content is preferably 1.0 mass% or less, more preferably 0.8 mass% or less, and even more preferably 0.6 mass% or less.

### [P: preferably more than 0 mass% and 0.1 mass% or less]

P is an element inevitably present as an impurity element. When the P content is excessive, weldability may be deteriorated. Therefore, the P content is preferably controlled to be 0.1 mass% or less, more preferably 0.08 mass% or less, and even more preferably 0.05 mass% or less.

### [S: preferably more than 0 mass% and 0.05 mass% or less]

S is an element inevitably present as an impurity element. Usually, steel inevitably contains S in an amount of about 0.0005 mass%. When the S content is excessive, a sulfide-based inclusion is formed, hydrogen absorption is promoted under a corrosive environment, delayed fracture resistance of the steel sheet is deteriorated, and the weldability and workability of the steel sheet may be deteriorated. Therefore, the S content is preferably controlled to be 0.05 mass% or less, more preferably 0.01 mass% or less, and even more preferably 0.005 mass% or less.

### [Al: preferably more than 0 mass% and 1.0 mass% or less]

Al is an element having a deoxidizing action. To allow such an action to be effectively exerted, the Al content is preferably more than 0 mass%, more preferably 0.005 mass% or more, and even more preferably 0.02 mass% or more. When the Al content is excessive, inclusions such as alumina increase, and the workability of the steel sheet may deteriorate. Therefore, the Al content is preferably 1.0 mass% or less, more preferably 0.8 mass% or less, and even more preferably 0.5 mass% or less.

### [N: preferably more than 0 mass% and 0.01 mass% or less]

N is an element inevitably present as an impurity element. When the N content is excessive, a nitride may be formed to deteriorate the workability of the steel sheet. In particular, when the steel sheet contains B for improving the hardenability, N bonds with B to form a BN precipitate, and inhibits the hardenability improving action of B. Therefore, the N content is preferably controlled to be 0.01 mass% or less, more preferably 0.008 mass% or less, and even more preferably 0.005 mass% or less.

### [Balance]

The balance is Fe and inevitable impurities. It is permitted to mix, as inevitable impurities, trace elements (e.g., As, Sb, and Sn) incorporated according to the conditions of raw materials, materials, manufacturing facilities, etc. It is usually preferable with P, S and N described above that the content is as small as possible, and therefore, these can be called inevitable impurities. However, the present disclosure is defined as described above because the effect of those elements can be easily exerted by controlling the contents of those elements to specific ranges. Thus, in the present description, "inevitable impurities" constituting the balance mean the concept excluding elements whose composition ranges are defined.

In addition to the above-described components, other well-known optional components can be further contained as long as the strength and sufficient bendability are not impaired. Examples of the optional components include Cu, Ni, Ti, Nb, V, and B. These optional components will be described below.

### [Cu: preferably more than 0 mass% and 1.0 mass% or less]

Similarly to Cr, Cu is an element that is effective for improving the strength of the steel sheet, has the action of suppressing the generation of hydrogen due to the corrosion of the steel sheet, and improves the corrosion resistance of the steel sheet. Similarly to Cr, Cu also has an action of promoting the production of iron oxide. To allow these actions to be effectively exerted, the Cu content is preferably more than 0 mass%, more preferably 0.003 mass% or more, and even more preferably 0.05 mass% or more. From the viewpoint of the workability of the steel sheet, the Cu content is preferably 1.0 mass% or less, more preferably 0.8 mass% or less, and even more preferably 0.5 mass% or less.

### [Ni: preferably more than 0 mass% and 1.0 mass% or less]

Similarly to Cr and Cu, Ni is an element that is effective for improving the strength of the steel sheet, has the action of suppressing the generation of hydrogen due to the corrosion of the steel sheet, and improves the corrosion resistance of the steel sheet. Ni also has an action of promoting the production of iron oxide similarly to Cr and Cu. To allow these actions to be effectively exerted, the Ni content is preferably more than 0 mass%, more preferably 0.003 mass% or more, and even more preferably 0.05 mass% or more. From the viewpoint of ensuring the workability of the steel sheet, the Ni content is preferably 1.0 mass% or less, more preferably 0.8 mass% or less, and even more preferably 0.5 mass% or less.

### [Ti: preferably more than 0 mass% and 0.15 mass% or less]

Similarly to Cr, Cu, and Ni, Ti is an element that is effective for improving the strength of the steel sheet, has the action of suppressing the generation of hydrogen due to the corrosion of the steel sheet, and improves the corrosion resistance of the steel sheet. Ti also has the action of promoting the production of iron oxide similarly to Cr, Cu, and Ni. In addition, because Ti is an element effective for the delayed fracture resistance of the steel sheet similarly to B and Cr, Ti may be contained in an amount at which the workability, such as strength or elongation, of the steel sheet is not affected. To allow these actions to be effectively exerted, the Ti content is preferably more than 0 mass%, more preferably 0.003 mass% or more, and even more preferably 0.05 mass% or more. From the viewpoint of ensuring the workability of the steel sheet, the Ti content is preferably 0.15 mass% or less, more preferably 0.12 mass% or less, and even more preferably 0.10 mass% or less.

### [Nb: preferably more than 0 mass% and 0.15 mass% or less]

Nb is an element that is effective for improving the strength of the steel sheet, and acts on improving the toughness of the steel sheet by miniaturizing austenite grains after quenching. To allow such actions to be effectively exerted, the Nb content is preferably more than 0 mass%, more preferably 0.003 mass% or more, and even more preferably 0.005 mass% or more. On the other hand, when the Nb content is excessive, a large amount of carbide, nitride, or carbonitride is generated, and the workability or delayed fracture resistance of the steel sheet may deteriorate. Therefore, the Nb content is preferably 0.15 mass% or less, more preferably 0.12 mass% or less, and even more preferably 0.10 mass% or less.

### [V: preferably more than 0 mass% and 0.15 mass% or less]

Similarly to Nb, V is also an element that is effective for improving the strength of the steel sheet, and acts on improving the toughness of the steel sheet by miniaturizing austenite grains after quenching. To allow such actions to be effectively exerted, the V content is preferably more than 0 mass%, more preferably 0.003 mass% or more, and even more preferably 0.005 mass% or more. On the other hand, when the V content is excessive, a large amount of carbide, nitride, or carbonitride is generated similarly to Nb, and the workability or delayed fracture resistance of the steel sheet may deteriorate. Therefore, the V content is preferably 0.15 mass% or less, more preferably 0.12 mass% or less, and even more preferably 0.10 mass% or less.

### [B: preferably more than 0 mass% and 0.005 mass% or less]

B is an element useful for improving the hardenability and weldability of the steel sheet. In addition, because B is an element effective for the delayed fracture resistance of the steel sheet similarly to Ti and Cr, B may be contained in an amount at which the workability, such as strength or elongation, of the steel sheet is not affected. To allow these actions to be effectively exerted, the B content is preferably more than 0 mass%, more preferably 0.0002 mass% or more, even more preferably 0.0003 mass% or more, and particularly preferably 0.0004 mass% or more. On the other hand, when the B content is excessive, such an effect may be saturated, and the ductility may be reduced to deteriorate the workability. Therefore, the B content is preferably 0.005 mass% or less, more preferably 0.004 mass% or less, and even more preferably 0.003 mass% or less.

Examples of the steel sheet include a cold rolled steel sheet and a plated steel sheet. The type of the plated steel sheet is not limited, and may be, for example, a zinc-based plated steel sheet provided with zinc-based plating, such as Al-Zn plating, Ni-Zn plating, Fe-Zn plating, Cr-Zn plating, or Mg-Zn plating. Specific examples of the zinc-based plated steel sheet include a galvanized steel sheet (GI), an alloyed galvanized steel sheet (GA), and an electrogalvanized steel sheet (EG).

### [Method for Manufacturing Steel Sheet]

Next, a method for manufacturing a high-strength steel sheet according to the present disclosure, especially a method for manufacturing a steel sheet having good platability will be described.

The method for manufacturing a steel sheet according to the present embodiment includes
an annealing step of performing an oxidation treatment under conditions of an oxygen concentration of 0.1 to 2% and an attainment temperature of 650 to 750°C and then performing a reduction treatment,
wherein the reduction treatment is performed through a first reduction treatment having a dew point of -35 to -15°C, and subsequently through a second reduction treatment having a dew point being -25 to 0°C and being higher than the dew point of the first reduction treatment.

By subjecting the surface of the steel sheet to an oxidation treatment, an Fe oxide layer is formed on the surface of the steel sheet. Next, by performing a reduction treatment in a reducing atmosphere, a reduced Fe layer capable of favorably forming, for example, a plating layer is formed on the steel sheet surface layer while a decarburized layer is formed. At this time, if water vapor is added throughout the reduction treatment, the decarburization amount becomes excessive, and the strength may decrease. On the other hand, when the dew point is set to a high dew point in the first half of the reduction treatment, decarburization is performed once, but carbon is re-diffused (recarburized) into the decarburized part in the latter half of the reduction treatment, so that the bendability is not improved. In view of this, the present inventors conducted studies, and resultantly have found that the decarburized state of the steel sheet surface layer portion, where both high strength and superior bendability can be attained, can be easily ensured by performing the oxidation treatment as described above, determining the dew point range of the first reduction treatment and that of the second reduction treatment in the reduction treatment, and making the dew point of the second reduction treatment higher than the dew point of the first reduction treatment. Hereinafter, the oxidation treatment and the reduction treatment will be described.

### (Oxidation Treatment)

The oxidation treatment is performed under the condition of an oxygen concentration of 0.1 to 2%. The oxidation treatment can be performed even under the condition of an oxygen concentration of 0.0%, but in the case of obtaining a plated steel sheet, the oxygen concentration is preferably set to 0.1% or more from the viewpoint of obtaining a superior plating appearance. The oxygen concentration is more preferably 0.15% or more, and even more preferably 0.20% or more. On the other hand, an excessively high oxygen concentration is prone to cause a defect called pick-up, which is a phenomenon in which an oxide scale adheres to a furnace roll due to excessive oxidation and a pressing mark occurs on a steel sheet. From the viewpoint of suppressing the occurrence of this defect, the oxygen concentration is set to 2% or less. The oxygen concentration is more preferably 1.7% or less, and even more preferably 1.5% or less. The concentration of elements other than oxygen is not particularly limited, and examples thereof include a gas atmosphere containing CO₂, N₂, H₂O, and other inevitable impurities together with oxygen having the above concentration. For example, the oxidation treatment can be performed in a combustion gas such as cokes oven gas (COG) or liquefied petroleum gas (LPG) in, for example, a direct fired furnace (DFF)-type annealing furnace or the like under a gas atmosphere in which a concentration of unburned O₂ is controlled.

The oxidation treatment is performed under the condition of an attainment temperature of 650 to 750°C. For example, the oxidation treatment may involve heating the steel sheet to an attainment temperature within a range of 650 to 750°C in an oxidation heating zone in a DFF-type annealing furnace. By setting the attainment temperature to 750°C or lower, it is possible to suppress a reaction particularly between SiO₂ on the steel sheet surface in the vicinity of the edge in the width direction of the steel sheet and FeO generated by the oxidation treatment. As a result, for example, when the steel sheet according to the present embodiment is a plated steel sheet, good plating adhesion can be obtained.

In the present description, the "attainment temperature" at the time of heating in the oxidation treatment means a maximum attainment sheet temperature of the steel sheet whose heating is controlled in an oxidation heating zone.

The attainment temperature in the oxidation treatment is preferably 730°C or lower, more preferably 720°C or lower, and even more preferably 700°C or lower. On the other hand, the steel sheet temperature in the oxidation treatment is set to 650°C or higher from the viewpoint of forming an Fe oxide layer in the gas atmosphere. The steel sheet temperature in the oxidation treatment is preferably 670°C or higher.

The temperature rise time in the oxidation treatment is not particularly limited, and may be adjusted such that, for example, a firelite layer that adversely affects the platability is not formed by the oxidation treatment due to an excessively long temperature rise time. Specifically, the temperature rise time in the oxidation treatment may be appropriately adjusted in consideration of the conditions of hot rolling (particularly the winding temperature), the annealing conditions before pickling, the pickling conditions, the temperature of the steel sheet during heating in the oxidation treatment, etc. The temperature rise time in the oxidation treatment is preferably 10 seconds or more, and more preferably 15 seconds or more, for example. In addition, the temperature rise time in the oxidation treatment is preferably 120 seconds or less, and more preferably 90 seconds or less, for example. Although the case where the oxidation treatment is performed while raising the temperature has been described above, the mode of the oxidation treatment is not limited thereto, and the oxidation treatment may be performed by raising the temperature up to the attainment temperature and holding the temperature at the attainment temperature.

### (Reduction Treatment)

In the reduction treatment, a desired decarburized layer is formed on the steel sheet surface layer. When the steel sheet is a plated steel sheet, a reduced Fe layer capable of favorably forming a plating layer is formed, for example. In the manufacturing method according to the present embodiment, the reduction treatment is performed through a first reduction treatment having a dew point of -35 to -15°C, and subsequently through a second reduction treatment having a dew point being -25 to 0°C and being higher than the dew point of the first reduction treatment. Hereinafter, each of the first reduction treatment and the second reduction treatment will be described.

### (First Reduction Treatment)

In the first reduction treatment, the dew point is set within a range of -35 to - 15°C. When the dew point is higher than -15°C, decarburization easily proceeds more than necessary, and the strength is easily deteriorated. In addition, the reduction treatment is less likely to proceed, and a defect called a pickup, in which iron oxide generated by the oxidation treatment adheres to a roll and causes a pressing mark on the steel sheet, is prone to occur. Therefore, the dew point is set to -15°C or lower. The dew point is preferably -20°C or lower. On the other hand, from the viewpoint of suppressing additional facilities and cost, the dew point in the first reduction treatment is set to -35°C or higher. The dew point is preferably -30°C or higher.

The dew point may satisfy the fact that the dew point in the atmosphere at the central portion of the front stage of the reduction zone where the first reduction treatment is performed is within the above range. The control of the dew point in the first reduction treatment and the second reduction treatment which is described later can be performed by, for example, a method in which a water vapor gas is charged and mixed with an atmospheric gas contained in a furnace, or a method in which an atmospheric gas is bubbled and water vapor is mixed.

The atmosphere of the first reduction treatment may be an atmosphere that satisfies the dew point described above and contains N₂, H₂, CO, H₂O, O₂, and other inevitable impurities. In the first reduction treatment, for example, the attainment temperature of the steel sheet reaches 800°C in the atmosphere described above, and then, the steel sheet is held in a temperature range of 800 to 920°C, for 60 to 240 seconds, for example. The term "hold" includes not only a case where the temperature is kept at a certain fixed temperature, but also a case where the temperature varies within the temperature range described above.

### (Second Reduction Treatment)

Next, the dew point of the second reduction treatment will be described. Fig. 1-1 (Nos. 1 to 16) and Fig. 1-2 (Nos. 17 to 22) are graphs created using Examples described later, and are graphs showing the relationship between the dew point at the center of the soaking zone during the second reduction treatment and R/t. From Figs. 1-1 and 1-2, it is found that the dew point in the second reduction treatment needs to be set to -25°C or higher in order to achieve superior bendability with a R/t of less than 2.5 as indicated by arrows in the diagrams. In addition, Fig. 2-1 (Nos. 1 to 16) and Fig. 2-2 (Nos. 17 to 22) are graphs created using Examples described later, and are graphs showing the relationship between the dew point at the center of the soaking zone during the second reduction treatment and the tensile strength TS. From Figs. 2-1 and 2-2, it is found that when the dew point is set to 0°C or lower, high strength with a tensile strength TS of 980 MPa or more, or 1180 MPa or more can be ensured. The dew point in the second reduction treatment is preferably -15°C or lower.

The atmosphere of the second reduction treatment may be an atmosphere that satisfies the dew point described above and contains N₂, H₂, CO, H₂O, O₂, and other inevitable impurities. In the second reduction treatment, for example, the steel sheet is held in the atmosphere described above within a temperature range in which the attainment temperature of the steel sheet is 800 to 920°C for 60 to 240 seconds, for example. The term "hold" includes not only a case where the temperature is kept at a certain fixed temperature, but also a case where the temperature varies within the temperature range described above.

The first reduction treatment and the second reduction treatment are merely required to be divided into atmospheres differing in dew point as described above, and their specific modes are not limited. For example, there may be provided reducing furnaces for performing the first reduction treatment and the second reduction treatment, respectively. When the steel sheet is a plated steel sheet, in the middle of the reduction zone of a continuous hot-dip plating line, a front region for performing the first reduction treatment and a rear region for performing the second reduction treatment may be separated by installing a partition wall having an opening area ratio of 20% or less, for example.

Between the first reduction treatment and the second reduction treatment, a step such as a holding step of holding at least any one of the conditions (dew point, heating temperature) of the first reduction treatment, for example, a cooling step of cooling to a temperature between the heating temperature of the first reduction treatment and room temperature may also be provided as long as there is no adverse effect on ensuring the decarburized state of the steel sheet according to the present embodiment. Preferably, the second reduction treatment is performed subsequently to the first reduction treatment.

The oxidation treatment and the reduction treatment may be performed using any publicly-known single facility or multiple facilities. Preferably, a facility of a continuous galvanizing line (CGL) is used from the viewpoint of manufacturing efficiency, cost, and quality retention. By using a continuous galvanizing line, an oxidation treatment and a reduction treatment by an oxidation-reduction method, and for example, a galvanizing treatment and an alloying treatment when a zinc-plated steel sheet is manufactured as the steel sheet, for example, can be continuously performed in a tandem manufacturing line. More specifically, the oxidation treatment and the reduction treatment by the oxidation-reduction method may be performed using, for example, an annealing furnace in a DFF-type continuous galvanizing line. For example, as described above, the oxidation treatment may be performed in a heating zone in a DFF-type annealing furnace. The reduction treatment may be performed, for example, in a soaking zone in a DFF-type annealing furnace.

The method for producing the steel sheet (substrate) to be subjected to annealing is not particularly limited. The steel sheet (substrate) to be subjected to annealing can be obtained by smelting and casting steel by a method usually performed to obtain a steel slab, and subjecting the steel slab to a rolling step (hot rolling, cold rolling) by a method usually performed.

The manufacturing method according to the present embodiment is merely required to include the annealing step, and the other steps are not limited. The steel sheet according to the present embodiment may be an annealed cold rolled steel sheet without undergoing any steps after the annealing. Alternatively, for example, a galvanizing treatment step and further an alloying treatment step may be provided as plating steps after annealing, and, for example, a galvanized steel sheet (GI) and an alloyed galvanized steel sheet (GA) may be obtained as the steel sheet according to the present embodiment. Alternatively, an electrogalvanized steel sheet (EG) may be obtained as the steel sheet according to the present embodiment by providing an electrogalvanizing treatment step.

The method for forming a galvanized layer on the surface of the annealed steel sheet is not particularly limited, and a publicly-known method can be appropriately used. For example, the base material after the annealing step is immersed in a plating bath. When the base material is immersed in the plating bath, it is preferable to control the plating deposition amount to, for example, 20 g/m² or more and 200 g/m² or less by, for example, gas wiping.

For example, binary or higher alloy plating containing Zn can be used for the plating bath. Examples of the binary or higher alloy plating containing Zn include Al-Zn plating, Fe-Zn plating, Ni-Zn plating, Cr-Zn plating, and Mg-Zn plating.

The plating may be performed by using a plating bath containing components other than zinc at a concentration of, for example, 0.01 mass% or more and 0.5 mass% or less and immersing a substrate in the plating bath at, for example, a temperature of 300°C or more and 600°C or less for 1 second or more and 30 seconds or less, for example. The alloying treatment is also not particularly limited, and a publicly-known method can be appropriately used. The alloying treatment may be performed, for example, by reheating at an alloying temperature of 470°C or more and 600°C or less for 1 second or more and 100 seconds or less.

### EXAMPLES

In the following, the present disclosure will be described more specifically with reference to Examples. The present disclosure is not limited by the following Examples, and can be implemented with appropriate modifications as long as the modifications can be consistent with the above-described and later-described gist, and all of them are included in the technical scope of the present disclosure.

As samples for the annealing, in Nos. 1 to 11, a substrate was prepared in which the component composition was a bulk carbon concentration, that is, a C content of the steel sheet (substrate) was 0.22 mass%, the Si content was 1.7 mass%, the Mn content was 2.0 mass%, the Cr content was 0.5 mass%, the Al content was 0.04 mass%, and the balance was Fe and inevitable impurities (note that the "inevitable impurities" referred to here included P, S, and N in amounts within the above-described ranges), the structure was ferrite + pearlite, and the strength was 700 to 800 MPa. In Nos. 12 to 16, a substrate was prepared in which the bulk carbon concentration was 0.13 mass% (0.13 mass% C), the Si content was 0.9 mass%, the Mn content was 2.3 mass%, the Cr content was 0.57 mass%, the Al content was 0.02 mass%, the balance was Fe and inevitable impurities (note that the "inevitable impurities" referred to here included P, S, and N in amounts within the above-described ranges), the structure was ferrite + pearlite, and the strength was 700 to 800 MPa. In Nos. 17 to 22, a substrate was prepared in which the bulk carbon concentration was 0.21 mass% (0.21 mass% C), the Si content was 1.8 mass%, the Mn content was 2.3 mass%, the Al content was 0.45 mass%, and the balance was Fe and inevitable impurities (note that the "inevitable impurities" referred to here included P, S, and N in amounts within the above-described ranges), the structure was ferrite + pearlite, and the strength was 600 to 700 MPa.

The samples for annealing described above were subjected to an oxidation treatment and a reduction treatment using an actual machine. Specifically, the oxidation treatment was performed at the oxygen concentration and the attainment temperature shown in Table 1, and then the first reduction treatment (heating zone) and the second reduction treatment (soaking zone) shown in Table 1 were performed in this order under each condition shown in Table 1 (attainment temperature, dew point). In Table 1, the conditions of the "first reduction zone" indicate the conditions of the first reduction treatment, and the conditions of the "second reduction zone" indicate the conditions of the second reduction treatment.

The steel sheet after the second reduction treatment was cooled to 460°C, and then immersed in an Al-Zn plating bath containing 0.08 to 0.13 mass% of Al (Al was effective Al%, and the plating bath temperature was 460 to 480°C) to perform zinc plating. The deposition amount of plating was controlled to 40 g/m² or more and 90 g/m² or less by gas wiping, and then an alloying treatment was performed at 480 to 490°C for 20 to 30 seconds, affording an alloyed galvanized steel sheet.

**[Table 1]**

| No. | Sheet thickness (mm) | Oxidation treatment | | Reduction treatment | | | |
|---|---|---|---|---|---|---|---|
| | | Oxygen concentration (%) | Ultimate temperature (°C) | First reduction zone ultimate temperature (°C) | First reduction zone dew point (°C) | Second reduction zone ultimate temperature (°C) | Second reduction zone dew point (°C) |
| 1 | 1.4 | 0.2 | 673 | 901 | -36.0 | 892 | -29.5 |
| 2 | 1.4 | 0.1 | 681 | 918 | -32.9 | 893 | -33.8 |
| 3 | 1.4 | 0.1 | 676 | 918 | -33.1 | 893 | -33.7 |
| 4 | 1.4 | 0.0 | 674 | 902 | -39.8 | 916 | -27.1 |
| 5 | 1.4 | 0.0 | 665 | 900 | -24.1 | 910 | -2.8 |
| 6 | 1.4 | 0.0 | 675 | 888 | -28.6 | 897 | -10.8 |
| 7 | 1.4 | 0.0 | 695 | 893 | -28.8 | 896 | -10.3 |
| 8 | 1.4 | 0.0 | 695 | 901 | -26.7 | 913 | -9.9 |
| 9 | 1.4 | 0.3 | 697 | 894 | -21.9 | 903 | -8.5 |
| 10 | 1.4 | 0.1 | 711 | 899 | -25.0 | 914 | -9.9 |
| 11 | 1.6 | 0.1 | 697 | 907 | -26.5 | 904 | -11.0 |
| 12 | 1.2 | 1.0 | 701 | 893 | -15.4 | 908 | -2.8 |
| 13 | 1.2 | 0.1 | 695 | 859 | -19.0 | 862 | -8.3 |
| 14 | 1.2 | 0.5 | 712 | 859 | -17.9 | 858 | -9.3 |
| 15 | 1.4 | 0.2 | 692 | 869 | -17.0 | 869 | -10.7 |
| 16 | 1.4 | 0.2 | 706 | 868 | -17.9 | 864 | -12.2 |
| 17 | 1.0 | 0.1 | 694 | 879 | -21.6 | 878 | -13.5 |
| 18 | 1.0 | 0.1 | 701 | 840 | -22.7 | 847 | -12.0 |
| 19 | 1.0 | 0.1 | 692 | 845 | -23.8 | 845 | -15.6 |
| 20 | 1.0 | 0.1 | 721 | 838 | -24.3 | 840 | -21.4 |
| 21 | 1.0 | 0.1 | 705 | 833 | -25.1 | 836 | -16.3 |
| 22 | 1.0 | 0.0 | 668 | 829 | -23.8 | 841 | -55.0 |

The obtained alloyed galvanized steel sheet was evaluated as follows.

### [Means for Measuring Decarburization Behavior: Measurement of Carbon Profile by GD-OES]

As described below, the carbon profile was measured by glow discharge optical emission spectrometry (GD-OES), and the decarburization behavior was examined.

### (Preparation of Sample)

A material having a size of 50 mm × 40 mm × plate thickness or 30 mm × 30 mm × plate thickness was taken. Thereafter, degreasing was performed in accordance with a conventional method, whereby a sample was prepared. Then, using this sample, the concentration in mass% of each element was measured by GD-OES under the following conditions.

### (Measurement Conditions)

Device used: Marcus-type high-frequency glow discharge optical emission spectroscopy (rf-GD-OES) GD-Profiler2 manufactured by HORIBA, Ltd.
Sputtering method: normal sputtering
Measurement range: φ 4 mm
Type of gas: Ar
Elements to be analyzed: B, C, O, Al, Si, Ti, Cr, Mn, Fe, Zn, P, S, and N
(In this example, these elements were evaluated, but when elements other than the above elements were contained in, for example, a plating layer or a steel sheet, elements other than the above elements were also to be analyzed.)

### (Measurement Method)

The surface of the sample on which the plating was formed was subjected to GD-OES measurement up to a depth of 150 µm in the sheet thickness direction.

### (Analysis Method)

Since the sputtering rate of the above device was substantially constant, the sputter crater depth of the sample after the analysis was measured, and the measured value (sputtering depth) was plotted in the horizontal axis.

Details of the calibration curve method for converting the measured emission intensity of each element into a concentration will be described as follows.

The relationship between the sputtering weight Wᵢ (g/sec) per unit time of the element i and the emission intensity Iᵢ is expressed by the following Equation (1) using the slope a and the intercept b of the calibration curve. ${W}_{i} = {aI}_{i} + b$

For the reference sample with which the concentration Cᵢ (wt%), the density ρ (g/cm³), and the sputtering rate Δd (cm/sec) are known, the sputtering weight Wᵢ per unit time of the element i is determined by the following Equation (2) using the sputtering area S (cm²). ${W}_{i} = {C}_{i} \times ρ \times Δd \times S$

The emission intensity Iᵢ was measured using two or more reference samples with known Wᵢ, and the slope a and the intercept b of the above Equation (1) were determined, and thus a calibration curve was prepared in which the horizontal axis was the emission intensity and the vertical axis was the sputtering weight. The reference samples used are shown in Table 2 below. Using the prepared calibration curve, the sputtering weight was determined from the emission intensity of each target element, and their weight ratios were converted into concentrations. The calibration curve used for the conversion of the O concentration was corrected using SiO₂ such that the concentration ratio of Si and O was 1 : 2.

**[Table 2]**

| **Reference sample** | **Main component** | **B** | **C** | **O** | **Al** | **Si** | **Ti** | **Cr** | **Mn** | **Fe** | **Zn** |
|---|---|---|---|---|---|---|---|---|---|---|---|
| BAS 113 | Fe | 0.0066 | 0.837 | - | 0.0151 | 0.931 | 0.039 | 1.248 | 1.207 | 94.99 | - |
| BAS 114 | Fe | 0.0008 | 0.403 | - | 0.078 | 0.295 | 0.0096 | 0.187 | 0.416 | 96.47 | - |
| MBH 13X NSD1 | Fe | - | 0.046 | - | 0.013 | 0.411 | - | 24.51 | 23.53 | 49.09 | - |
| MBH 13X 8110L | Fe | (1.09) | 0.792 | - | 0.009 | 0.96 | 0.055 | 12.33 | 0.772 | 76.08 | - |
| MBH 31X BIB3 | Cu | - | - | - | 0.0298 | 0.061 | - | - | 0.243 | 0.099 | 32.46 |
| SPEX 185-CO2 | Cu | - | - | - | - | - | - | - | - | 0.096 | 0.15 |
| Japan Fine Ceramics Co., Ltd. Al2O3 | O | - | - | 47.07 | (52.93) | - | - | - | - | - | - |

| | | | | | | | | | | | |
|---|---|---|---|---|---|---|---|---|---|---|---|
| * The numeral value in the parenthesis in the table was excluded from the reference value to be used for concentration conversion. | | | | | | | | | | | |

Then, a carbon profile was obtained using the analysis result on carbon. One example thereof is illustrated in Fig. 3. Fig. 3 illustrates No. 2, which is a comparative example, and No. 10, which is an example of the present invention. In Fig. 3, it can be seen that the carbon profiles of both the materials each has a peak of the carbon concentration within 20 µm of the surface layer (specifically, in the internal oxide layer), but the carbon concentration is higher than the bulk carbon concentration in the comparative example, whereas the carbon concentration is sufficiently lower than the bulk carbon concentration in the present invention example. Since the bulk carbon concentration of the sample used in this example was 0.22 mass%, the upper limit of the maximum value (vertical axis) of the carbon concentration (mass%) in the region up to 20 µm from the steel sheet surface is 0.22 mass% × 70% = 0.15 mass%.

From the obtained carbon concentration profile in the sheet thickness direction, the position where the carbon concentration (mass%) was 50% of the bulk carbon concentration, the position where the carbon concentration (mass%) was 90% of the bulk carbon concentration, and the maximum value of the carbon concentration (mass%) in the region up to 20 µm from the steel sheet surface were determined. The bulk carbon concentration was corrected such that the carbon concentration at a sufficiently deep position (120 to 150 µm) measured by GD-OES equaled a value obtained by ordinary steel analysis, and then the corrected value was used for analysis. For example, when the steel analysis value was 0.22% and the analysis value by GD-OES was 0.25%, the analysis value by GD-OES was multiplied by 0.22/0.25 and then used for analysis.

The surface layer decarburization amount per millimeter of the sheet thickness on one surface of the steel sheet was determined as follows. First, the amount of desorbed carbon was determined from the difference between the bulk carbon concentration and the carbon concentration profile of the steel sheet (after decarburization). That is, for a 1m² steel sheet, the total decarburization amount was determined from the volume (m³) of iron in the decarburized part × the density (specific gravity) of iron (7.87 × 10⁶ g/m³) × the ratio of decarburized carbon accounting for in the iron in the decarburized part/the atomic weight (g/mol) of carbon. Then, the total decarburization amount was divided by the sheet thickness, whereby the surface layer decarburization amount (mol/m²) per millimeter of the sheet thickness of one steel sheet surface was determined.

### [Evaluation of Critical Bendability (R/t)]

The bendability of a steel sheet was evaluated by the following procedure. A test piece having a width of 40 mm and a length of 100 mm with a long axis in a direction perpendicular to the rolling direction was prepared, and a bending test was performed by a V block method in accordance with JIS Z 2248:2014. In the bending test, the bending radius was varied from 0 to 7 mm, the minimum bending radius at which the material could be bent without being broken was determined. Then, using this as the critical bending radius R (mm), the critical bending radius R (mm)/sheet thickness t (mm) ratio was calculated. Then, a case where the critical bending radius R (mm)/sheet thickness t (mm) was less than 2.5 was evaluated as being superior in bendability, whereas a case where the critical bending radius R (mm)/sheet thickness t (mm) was 2.5 or more was evaluated as being poor in bendability.

### [Measurement of Tensile Strength (TS)]

The tensile strength (TS) was measured in accordance with the method specified in JIS Z 2241:2011 by taking a JIS No. 5 tensile test piece from a steel sheet such that a direction perpendicular to the rolling direction of the steel sheet was the longitudinal direction. Then, a case where the tensile strength (TS) was 980 MPa or more was evaluated as being high in strength (preferably, a case where the TS was 1180 MPa or more was evaluated as being higher in strength), whereas a case where the TS was less than 980 MPa was evaluated as being poor in strength.

### [Evaluation of Platability]

The appearance of a plated steel sheet sample was visually observed. Then, a case where adhesion of dross caused by the presence of selective oxides of Si and Mn adversely affecting plating formation was confirmed was evaluated as being inferior in platability (×), whereas a case where adhesion of dross was not confirmed was evaluated as being superior in platability (∘). The results are shown in Table 3.

**[Table 3]**

| No. | Analysis results | | | | | | |
|---|---|---|---|---|---|---|---|
| | (1) Position with 50% of bulk carbon (% accounting for in sheet thickness) | (2) Position with 90% of bulk carbon (% accounting for in sheet thickness) | (3) Ratio (%) of maximum value of carbon concentration (mass%) in region up to 20 µm from steel sheet surface (%) | (4) Surface layer decarburization amount (mol/m²) per millimeter of sheet thickness (mol/m²) (up to 0.9C) | (5) Bending R/t | (6)TS (MPa) | Plating property |
| 1 | 0.18 | 5.4 | 84.8 | 0.018 | 3.2 | 1232 | ○ |
| 2 | 0.03 | 5.2 | 98.2 | 0.013 | 3.2 | 1230 | ○ |
| 3 | 0.17 | 5.9 | 88.3 | 0.019 | 2.5 | 1221 | ○ |
| 4 | 0.00 | 3.9 | 89.0 | 0.009 | 2.5 | 1223 | × |
| 5 | 1.88 | 5.7 | 39.0 | 0.032 | 1.1 | 1193 | × |
| 6 | 0.27 | 4.6 | 61.0 | 0.021 | 1.4 | 1212 | × |
| 7 | 0.28 | 4.8 | 50.4 | 0.022 | 1.8 | 1222 | × |
| 8 | 0.22 | 5.3 | 60.0 | 0.023 | 1.8 | 1211 | × |
| 9 | 2.16 | 6.8 | 42.4 | 0.034 | 1.1 | 1214 | ○ |
| 10 | 0.25 | 5.3 | 64.2 | 0.022 | 1.8 | 1207 | ○ |
| 11 | 1.61 | 6.3 | 38.0 | 0.031 | 2.2 | 1222 | ○ |
| 12 | 2.74 | 7.8 | 36.4 | 0.045 | 1.7 | 1199 | ○ |
| 13 | 1.75 | 5.4 | 48.3 | 0.017 | 1.5 | 1216 | ○ |
| 14 | 2.49 | 6.4 | 36.1 | 0.023 | 1.5 | 1221 | ○ |
| 15 | 2.14 | 5.7 | 41.2 | 0.020 | 1.5 | 1231 | ○ |
| 16 | 2.04 | 5.6 | 40.9 | 0.019 | 1.5 | 1244 | ○ |
| 17 | 2.96 | 6.7 | 27.9 | 0.043 | 0.0 | 998 | ○ |
| 18 | 2.92 | 6.8 | 33.8 | 0.042 | 0.0 | 1009 | ○ |
| 19 | 1.85 | 6.1 | 37.1 | 0.032 | 0.0 | 1000 | ○ |
| 20 | 1.65 | 6.1 | 49.0 | 0.032 | 0.0 | 1033 | ○ |
| 21 | 2.25 | 6.5 | 45.4 | 0.035 | 0.0 | 1013 | ○ |
| 22 | 0.01 | 0.1 | 117.6 | 0.000 | 2.5 | 1099 | × |

On the basis of the results of Table 3 above, graphs showing the relationship between the position where the carbon concentration (mass%) in the sheet thickness direction is 50% of the bulk carbon concentration and R/t are shown in Fig. 4-1 (Nos. 1 to 16) and Fig. 4-2 (Nos. 17 to 22). From Figs. 4-1 and 4-2, it can be seen that to achieve superior bendability with which R/t is less than 2.5 as indicated by the arrow in the diagram, the position where the carbon concentration (mass%) in the sheet thickness direction is 50% of the bulk carbon concentration may be in a region of 0.20% or more of the sheet thickness from the steel sheet surface.

On the basis of the results of Table 3 above, graphs showing the relationship between the position where the carbon concentration (mass%) in the sheet thickness direction is 90% of the bulk carbon concentration and the tensile strength TS are shown in Fig. 5-1 (Nos. 1 to 16) and Fig. 5-2 (Nos. 17 to 22). From Figs. 5-1 and 5-2, it can be seen that when the position where the carbon concentration (mass%) in the sheet thickness direction is 90% of the bulk carbon concentration is in a region of 8.0% or less of the sheet thickness from the steel sheet surface, high strength with a tensile strength TS of 980 MPa or more, preferably 1180 MPa or more can be ensured.

On the basis of the results in Table 3 above, graphs showing the relationship between the ratio of the maximum value of the carbon concentration (mass%) in the region up to 20 µm from the steel sheet surface to the bulk carbon concentration and R/t are shown in Fig. 6-1 (Nos. 1 to 16) and Fig. 6-2 (Nos. 17 to 22). From Figs. 6-1 and 6-2, it can be seen that to achieve superior bendability with which R/t is less than 2.5 as indicated by the arrow in the diagram, the ratio of the maximum value of the carbon concentration (mass%) in the region up to 20 µm from the steel sheet surface to the bulk carbon concentration is preferably set to less than 70%.

On the basis of the results of Table 3 above, graphs showing the relationship between the surface layer decarburization amount per millimeter of the sheet thickness on one steel sheet surface and the tensile strength TS are shown in Fig. 7-1 (Nos. 1 to 16) and Fig. 7-2 (Nos. 17 to 22). From Figs. 7-1 and 7-2, it can be seen that when the surface layer decarburization amount per millimeter of the sheet thickness is 0.045 mol/m² or less, preferably 0.035 mol/m² or less, high strength represented by a tensile strength TS of 980 MPa or more, preferably 1180 MPa or more can be secured. Preferably, when the surface layer decarburization amount per millimeter of the sheet thickness is adjusted to 0.028 mol/m² or less, a higher tensile strength TS of 1200 MPa or more can be achieved.

In Table 3, Nos. 1 to 4 and 22 had no surface layer portion of a steel sheet defined in the present embodiment, and were inferior in bendability. Nos. 5 to 21 each had a surface layer portion of a steel sheet defined in the present embodiment, and were able to achieve both high strength and superior bendability. In addition, as characteristics of a steel sheet, it can be seen that to ensure not only high strength and superior bendability but also superior platability, the oxidation treatment is preferably performed under prescribed conditions in the manufacturing process as in Nos. 9 to 21.

The disclosure in this description may include the following aspects.

Aspect 1 of the present invention is
a steel sheet, wherein, in a sheet thickness direction,
a position where a carbon concentration (mass%) is 50% of a bulk carbon concentration is in a region of 0.20% or more of the sheet thickness from a steel sheet surface, and
a position where a carbon concentration (mass%) is 90% of the bulk carbon concentration is in a region of 8.0% or less of the sheet thickness from the steel sheet surface.

Aspect 2 of the present invention provides
the steel sheet according to Aspect 1, wherein a maximum value of a carbon concentration (mass%) in a region up to 20 µm in the sheet thickness direction from a steel sheet surface is less than 70% of the bulk carbon concentration, and
a surface layer decarburization amount per millimeter of the sheet thickness on one surface of the steel sheet is 0.035 mol/m² or less.

Aspect 3 of the present invention provides
the steel sheet according to Aspect 1 or 2, wherein
the steel sheet has a tensile strength of 1180 MPa or more.

Aspect 4 of the present invention provides
the steel sheet according to any one of Aspects 1 to 3, wherein a component composition satisfies:
C: 0.08 mass% or more and 0.30 mass% or less;
Si: more than 0.5 mass% and 3.0 mass% or less;
Mn: 1.5 mass% or more and 3.0 mass% or less;
Cr: more than 0 mass% and 1.0 mass% or less;
P: more than 0 mass% and 0.1 mass% or less;
S: more than 0 mass% and 0.05 mass% or less;
Al: more than 0 mass% and 1.0 mass% or less; and
N: more than 0 mass% and 0.01 mass% or less,
with the balance being Fe and inevitable impurities.

Aspect 5 of the present invention is
a method for manufacturing a steel sheet, the method comprising an annealing step of performing an oxidation treatment under conditions of an oxygen concentration of 0.1 to 2% and an attainment temperature of 650 to 750°C and then performing a reduction treatment,
wherein the reduction treatment is performed through a first reduction treatment having a dew point of -35 to -15°C, and subsequently through a second reduction treatment having a dew point being -25 to 0°C and being higher than the dew point of the first reduction treatment.

Aspect 6 of the present invention is
the method for manufacturing a steel sheet according to Aspect 5, wherein an attainment temperature in the first reduction treatment and the second reduction treatment is 800 to 920°C.

This application claims priority based on Japanese Patent Application No. 2023-056165 filed on March 30, 2023 and priority based on Japanese Patent Application No. 2024-022770 filed on February 19, 2024. Japanese Patent Application Nos. 2023-056165 and 2024-022770 are incorporated herein by reference.

## Claims

1. A steel sheet, wherein, in a sheet thickness direction,
a position where a carbon concentration (mass%) is 50% of a bulk carbon concentration is in a region of 0.20% or more of the sheet thickness from a steel sheet surface, and
a position where a carbon concentration (mass%) is 90% of the bulk carbon concentration is in a region of 8.0% or less of the sheet thickness from the steel sheet surface.

2. The steel sheet according to claim 1, wherein a maximum value of a carbon concentration (mass%) in a region up to 20 µm in the sheet thickness direction from a steel sheet surface is less than 70% of the bulk carbon concentration, and
a surface layer decarburization amount per millimeter of the sheet thickness on one surface of the steel sheet is 0.045 mol/m² or less.

3. The steel sheet according to claim 1 or 2, wherein the steel sheet has a tensile strength of 980 MPa or more.

4. The steel sheet according to claim 1 or 2, wherein a component composition satisfies:
C: 0.08 mass% or more and 0.30 mass% or less;
Si: more than 0.5 mass% and 3.0 mass% or less;
Mn: 1.5 mass% or more and 3.0 mass% or less;
Cr: 0 mass% or more and 1.0 mass% or less;
P: more than 0 mass% and 0.1 mass% or less;
S: more than 0 mass% and 0.05 mass% or less;
Al: more than 0 mass% and 1.0 mass% or less; and
N: more than 0 mass% and 0.01 mass% or less,
with the balance being Fe and inevitable impurities.

5. A method for manufacturing a steel sheet, the method comprising an annealing step of performing an oxidation treatment under conditions of an oxygen concentration of 0.1 to 2% and an attainment temperature of 650 to 750°C and then performing a reduction treatment,
wherein the reduction treatment is performed through a first reduction treatment having a dew point of -35 to -15°C, and subsequently through a second reduction treatment having a dew point being -25 to 0°C and being higher than the dew point of the first reduction treatment.

6. The method for manufacturing a steel sheet according to claim 5, wherein an attainment temperature in the first reduction treatment and the second reduction treatment is 800 to 920°C.
